

## UNITED STATES PATENT OFFICE

HERMANN HECKEL, OF CINCINNATI, OHIO, ASSIGNOR TO THE TWITCHELL PROCESS COMPANY, OF ST. BERNARD, OHIO, A CORPORATION OF OHIO

## FLEXIBLE TRANSPARENT GELATINOUS PRODUCT

No Drawing.

Application filed May 5, 1931. Serial No. 535,303.

This invention relates to flexible transparent gelatinous products such as gelatin sheets and likewise to a process of making them.

In my copending application Serial No. 5 432,565 I have disclosed and claimed the use of an admixture of mahogany sulphonates and oil as a softening agent for glues, gelatins, and like products in order to render them more flexible and have fully set forth 10 the advantages of said softening agents over softening agents previously used.

The object of this invention is to provide a process of making gelatinous products such as gelatin sheets both flexible and transparent with the use of mahogany sulphonates and oil as a softening agent.

It is likewise the object of the invention to provide improved gelatinous products which are both transparent and flexible. The 20 mahogany sulphonates in question are particularly described in the Fischer and Reddish Patent No. 1,703,838, February 26, 1929. The oil which I prefer to use for the purposes of this invention is a transparent one 25 of the type known as medicinal white oil. The invention will be disclosed particularly in relation to the manufacture of gelatin sheets.

A water solution is first made containing 30 between 5 and 15% gelatin. Next is added the softening agent which may be in quantity up to 35% the weight of the gelatin depending on the flexibility desired. A 20 to 25% proportion of softener to gelatin is considered appropriate and expedient for gelatin sheets. The softener, that is, the mahogany sulphonates and the oil, tend to form the milky or turbid solution in the gelatin solution and this lack of full and complete transparency is undesirable in the ultimate product.

To counteract this tendency toward cloudiness, I use in the softener and/or in the solution, between 10 and 20% of a substance 45 adapted to clarify the solution. The substances which have given good results comprise methanol, ethanol, butyl cello solve and hexalin. These bodies may be added directly to the softener or to the solution. The 50 softener itself may comprise between 30 and

45% mahogany sulphonates and between 70 and 55% oil. The admixture of 45% mahogany sulphonates, 55% oil and 10% of their weight of hexalin produces a softener for gelatin films or sheets which is highly suitable for producing finished products adapted to be used as transparent wrapping paper.

The gelatin sheets or films are usually formed by flowing the gelatin solution upon a belt, evaporating the water and other volatile components such as the alcohol, drying the film, then stripping the film from the belt.

All claims directed to the emulsifying properties of mahogany sulphonates, the use of alcohols and the like in conjunction therewith and the softening action of mahogany and oil solutions on the colloidal bodies, are reserved for other copending applications, the subject matter being claimed herein being strictly limited to the product and method aspects 70 of forming flexible transparent gelatinous bodies.

Having described my invention, I desire to be limited only by the ensuing claims:

1. A transparent and flexible gelatinous 75 product, the constituting components of which comprise gelatin, white oil, and mahogany sulphonates.

2. The method of producing transparent flexible gelatinous products, said method, 80 comprising, forming a solution of gelatin in water, emulsifying transparent oil in said solution by using mahogany sulphonates as emulsifying agents, maintaining said solution clear by means of an alcohol therein, and forming the final product by evaporation of the volatile components.

3. The method of producing transparent flexible gelatinous products, said method, 85 comprising, forming a solution of gelatin in water, emulsifying transparent oil in said solution by using mahogany sulphonates as emulsifying agents, maintaining said solution clear by means of hexalin, and forming the final product by evaporation of the volatile components.

4. The method of producing transparent flexible gelatinous products, said method, 90 comprising, forming a solution of gelatin in water, emulsifying transparent oil in said so-

55

60

65

70

75

80

85

90

95

100

lution by using mahogany sulphonates as emulsifying agents, maintaining said solution clear by means of butyl cello solve, and forming the final product by evaporation of 5 the volatile components.

5. In the process of making transparent flexible gelatinous products, the step of forming a solution, the constituting components of which comprise water, gelatin, transparent 10 oil, mahogany sulphonates, and a volatile substance of the nature disclosed adapted to render said solution clear and transparent.

6. A transparent and flexible gelatinous product, comprising, gelatin and a softener 15 for the gelatin, comprising, mahogany sulphonates and white oil, said softener being approximately 20 to 25% of the weight of the gelatin.

In witness whereof, I hereunto subscribe 20 my name.

HERMANN HECKEL.

25

30

35

40

45

50

55

60

65